

3,341,931  
BRAKE SHOES

Herbert L. Libbin, New Shrewsbury, and Roswell S. Fritchette, Jr., Ramsey, N.J., and Howard B. Huntress, Suffern, N.Y., assignors to Abex Corporation, a corporation of Delaware

Continuation of application Ser. No. 313,799, Oct. 4, 1963. This application Nov. 10, 1965, Ser. No. 507,229  
5 Claims. (Cl. 29—420.5)

## ABSTRACT OF THE DISCLOSURE

A method of producing a superior railroad brake shoe, in the form of a sintered body of powdered metal including iron and graphite, by subjecting the sintered body to repeated pressure-no pressure cycles of the order of 3000 p.s.i. at an elevated temperature and in a time period of less than 1.5 minutes.

This invention relates to an improved railroad car brake shoe and, more particularly, to such a brake shoe formed by a sintering process and exhibiting improved mechanical properties such as desirable frictional properties as well as higher strength than previously attainable. This application is a continuation of application Ser. No. 313,799, filed Oct. 4, 1963, now abandoned.

In order to more clearly disclose the novel aspects of this invention, a brief discussion of the field of art to which it pertains is deemed to be pertinent. For a great many years, the only material used as the friction producing body to brake railroad cars was metallic in nature and was composed of cast ferrous alloys. These brake shoes have been usually provided with a steel back around and upon which the cast material has been founded. This may be illustrated, for example, by United States Patent No. 1,157,183. The vast majority of railroad cars operating in interchange service in the United States, Canada and Mexico are provided with such brake shoes.

More recently, improvements in the technology of forming and newly available materials have permitted the use of essentially organically bonded brake shoes to be used for certain types of railroad cars and in certain types of service. These so-called "composition" brake shoes have usually been composed of thermosetting resins, elastomers, asbestos fiber and certain other inorganic fillers and friction modifying agents.

Among many differences which exist between these two types of brake shoes, and perhaps the most important from a functional viewpoint, is the difference in their frictional properties. The cast metal brake shoe, when evaluated under conditions specified by the Association of American Railroads (A.A.R.), is required to possess a mean coefficient of friction of at least 0.15 and a wear rate not to exceed 3.85 cubic inches of brake shoe material per 100,000 foot pounds of energy absorbed in braking effort. Under similarly specified conditions, the composition brake shoe has a mean coefficient of friction of about 0.36 and a wear rate of about 0.5 cubic inch per 100,000 foot pounds. These properties are determined by testing brake shoes against a full size railroad car wheel mounted upon an appropriate dynamometer.

Because of these vastly different coefficients of friction, the brake rigging on a car equipped with composition brake shoes must be modified so that the load applied to these shoes during the braking action is much lower than that applied to the cast metal shoes. This is necessary to avoid serious trouble during the braking of a train, par-

ticularly in cases where some cars in the train are equipped with composition brake shoes and the others with cast metallic brake shoes. Because of this, it is readily apparent that care must be exercised in replacing worn brake shoes to prevent placing cast metal shoes on a car whose brake rigging has been modified for composition shoes, or equally dangerous, composition shoes on a car with standard rigging. In the first case, when the brakes are applied, inadequate braking action will take place. In the second case, the braking action is excessive to the point where the wheels may lock resulting in producing flat spots on the wheels, or, more drastically, in pulling the train apart with a possible derailment.

Over the many years of their use, the cast metal brake shoes have been exposed to practically every environmental condition it is possible to imagine and, except for normal wear during the braking function, has proven to be virtually indestructible. During the much briefer history of the composition brake shoe it has been found to be somewhat more prone to damage. In particular, one of the more troublesome properties of the composition shoe is its lack of resistance to fire. It is a common practice during winter in the northern states for railroad yard employees to use torches to thaw frozen or ice-covered portions of cars. If composition brake shoes are exposed to flames for very long, the organic material may be seriously damaged or destroyed; another cause of excessive wear and damage to composition shoes may originate in an excessively rough wheel tread surface. The composition material is relatively soft and such a tread condition will abrade it away at a relatively rapid rate, whereas the cast metal shoe is relatively immune.

For these and other reasons, it has become desirable to provide a brake shoe having the advantages inherent in the metallic brake shoe with those inherent in the composition brake shoe. Further, it is desirable that such an improved brake shoe be interchangeable with existing composition brake shoes without further modification of the braking systems of the not inconsiderable number of cars already modified for composition brake shoes. In addition, it would also be desirable to provide such a brake shoe with even higher frictional properties for new car construction.

It is therefore, a principal object of this invention to provide a railroad brake shoe having essentially metallic characteristics and higher friction properties than previously known cast metal brake shoes. A further object of this invention is the provision of such a brake shoe having a mean coefficient of friction at least as high as existing composition brake shoes. A yet further object of this invention is the provision of such a brake shoe composed essentially of sintered iron powders and powdered graphite which may include friction augmenting or modifying agents, which shoe, exhibits a higher mechanical strength than that previously producible. Other and different objects of this invention will become apparent from the following description, wherein it is to be understood that changes in the precise embodiment of the invention can be made within the scope of what is claimed without departing from the spirit thereof.

Briefly stated and in accordance with one aspect of the invention, a railroad car brake shoe is produced by sintering and hot forming a mixture of from about 60 to 75% by weight iron powder, from about 10 to 25% by weight powdered graphite and up to 20% by weight of friction modifying and augmenting agents under conditions to provide the brake shoe with a mean coefficient of friction of at least 0.30 and a wear rate of less than 3.85 cubic inches per 100,000,000 foot pounds of energy absorption, and having a transverse rupture strength of at least 3,000 pounds per square inch.

The following detailed description of the several compositions and methods employed in achieving such an improved and novel railroad car brake shoe are set forth for the purpose of more completely disclosing the various aspects of the invention and are merely exemplary and not to be construed as limiting the scope of the invention except as may be set forth in the several claims.

Essentially the inventive subject matter involves the provision of a railroad car brake shoe composed of a wrought and appropriately shaped steel back provided with lugs and guide members where desired to adapt it and the attached body or bodies of friction material to be mounted upon the brake head of a railroad car. In order for the improved brake shoe to accomplish the purposes and objects of the invention, the friction material attached to the steel back must have certain mechanical and frictional properties which are dependent upon its composition and the manner in which it is formed. As will be more specifically described subsequently, it has been found that such a brake shoe may be constructed by forming a plurality of steel backed segments of friction material and attaching them by bolting, riveting, or any appropriate means to a steel brake shoe which may then be attached to a brake head or, more desirably, by forming an integral mass of friction material in contact with and securely affixed to a steel brake shoe back as a single, monolithic structure to be attached to a brake head.

More specifically, appropriate proportions of iron powder, graphite and perhaps other pulverulent materials, as will be subsequently disclosed, are thoroughly mixed in the dry state, placed in an appropriately configured die and pressed at room temperature under loads of from about 5 tons per square inch to as high as about 14 tons per square inch to form a cold, compacted self-supporting body. The compacted powder body is then removed from the forming die and an appropriate steel back is assembled therewith and the two piece assembly is placed within a protective atmosphere furnace and heated to at least 1900° F. for about 1 hour. The assembled body and steel back are then removed from the furnace and placed immediately in an appropriately formed forming die and subjected to a cyclically applied pressure by means of a punch-like member which substantially fills and closes the upper open end portion of the die cavity. This loading is accomplished by applying a pressure of 3,000 pounds per square inch for 7.5 seconds and releasing the pressure for 1 second and then repeating the cycle for a total of 8 cycles. The composite body is then removed from the die and cooled. Preferably the cooling is done by inserting the body into a container of solid carbon dioxide (Dry Ice) whereby the rate of cooling is accelerated and a protective, non-oxidizing atmosphere is provided. The finished body is composed of a layer of compacted and sintered friction material securely fastened or welded to the steel back and suitable for use as a segmented railroad brake shoe, as previously described or, if the sintered friction material has been secured directly to a wrought steel railroad brake shoe back member, as a monolithic railroad brake shoe. The apparatus for accomplishing this is well known and a similar process is described and illustrated in United States Patent No. 2,892,707, hereinafter referred to as the Biggs patent. It should be noted, however, that the above-recited process differs in several important details from that disclosed in the Biggs patent. The patent discloses the use of a specifically different friction composition and, additionally, a much lower pressure and a substantially greater number of cycles employed during the pressing operation. As will be shown in greater detail, the pressure of 3,000 pounds per square inch and the significantly lower number of cycles utilized in the practice of this invention results in an unexpectedly higher transverse rupture strength and the composition

used has frictional properties which enable the resulting material to be used for railroad braking purposes.

It should be noted, particularly in view of the fact that the sintered powder metal friction material art is quite well developed, that when sintering such iron base materials under pressure, i.e. utilizing the application of pressure to the powder compact during the sintering operation, 1800° F. has proven to be quite adequate as a sintering temperature. Furthermore, in such materials the inclusion of as much as 20 percent by weight of lead powder in the compact has been shown to have virtually no effect upon the transverse rupture strength when compared to the same material without the lead.

#### Example 1

A mixture of dry powders having the following composition was prepared:

|                                 | Percent by weight |
|---------------------------------|-------------------|
| Iron powder (-40 mesh)          | 70.5              |
| Graphite powder (35 to 65 mesh) | 20.0              |
| Alundum powder (about 100 mesh) | 5.0               |
| Tin powder (about 325 mesh)     | 2.5               |
| Lead powder (about 325 mesh)    | 2.0               |

After thoroughly mixing the powders at room temperature, they were pressed at room temperature in a die at a pressure of 5 tons per square inch to form a self-sustaining compact having a configuration and approximate dimensions of a full-size standard railroad brake shoe. This compact was then removed from the die and a wrought steel brake shoe back placed upon it. The two so-assembled bodies were then placed in a furnace and heated for 1 hour at 1900° F. A protective atmosphere was generated in the furnace by the presence of charcoal therein. At the end of the 1 hour period, the compact and back were removed, still in the assembled relationship, and immediately placed in the hot forming die having the dimensions and configuration of a full-size railroad brake shoe and subjected to a cyclically applied compacting pressure of 3,000 pounds per square inch. The pressure cycle employed applied the 3,000 pounds per square inch load for 7.5 seconds and then released the load for 1 second. This cycle was repeated for a total of 8 such cycles. The so-formed brake shoe was then removed from the die and placed in a container with solid carbon dioxide blocks (Dry Ice) and permitted to cool. Subsequently, this brake shoe was mounted on a brake head in a dynamometer in which a standard railroad car wheel was installed and its frictional properties and wear rate was determined under standard A.A.R. specified conditions. In this test, an equivalent wheel load of 7,324 pounds, a brake shoe load of 2,500 pounds and a 36 inch diameter wheel were used. Under these conditions, the brake shoe produced a dynamometer stop distance of 800 feet or less from 60 miles per hour. After five preliminary stops to wear in or "seat" the brake shoe, the results of which were discarded, a series of 15 stops were made from 60 miles per hour. It was found from these tests that this brake shoe had a mean coefficient of friction of 0.49 and a wear rate of 1.11 cubic inches per 100,000,000 foot pounds of energy absorbed. Test specimens measuring 1" x 2" x 0.2" were cut from the sintered friction material portion of the brake shoe and subjected to a standard three point transverse rupture test. The material exhibited a transverse rupture strength of 4,060 pounds per square inch.

#### Example 2

A mixture of powders having a composition identical to that of Example 1 was mixed and processed in the same manner and by the same equipment as that of Example 1 except it and its associated steel back were heated for 1 hour at 1800° F. instead of 1900° F., and it was subjected to a hot forming operation consisting of 16 cycles of 1,500 pounds per square inch applied for 4 sec-

onds followed by a release of pressure for 1 second. In all other respects the brake shoe was identically treated to that produced in Example 1. It was subjected to the same testing procedure on the dynamometer and was found to have a mean coefficient of friction of 0.44 and a wear rate of 1.17 cubic inches per 100,000,000 foot pounds of absorbed energy. When similar test specimens were cut from the friction material of this brake shoe and subjected to the same transverse rupture strength test it was found to have a strength of only 2,540 pounds per square inch.

*Example 3*

A mixture of powders having a composition identical to that of Example 1 was mixed and processed in the same manner and by the same equipment as that of Example 1 except that the dies used produced flat plate-like or block-like bodies of sintered friction material about 7" long by 4½" wide by 1" thick having a 7" by 4½" by ¾" thick steel back secured to one face thereof. Additionally, a higher cold pressing pressure of 14 tons per square inch was employed. A plurality of these blocks were secured to a standard steel brake shoe back and trimmed and ground to present a wear face substantially identical in size and shape to that of the brake shoe of Example 1. When tested upon the dynamometer as set forth in Example 1, this segmental shoe was found to have a mean coefficient of friction of 0.40 and a wear rate of 0.43 cubic inch per 100,000,000 foot pounds. This friction material had a transverse rupture strength of 4,800 pounds per square inch.

*Example 4*

A mixture of powders having a composition identical to that of Example 1 was mixed and processed in the same manner and by the same equipment as that of Example 3 except that the heating temperature, hot forming pressure and pressure cycle set forth in Example 2 was used. Transverse rupture test specimens were cut from the friction material and upon test were found to have a transverse rupture strength of 2,540 pounds per square inch.

In order to illustrate the relationship and effect of the several variables upon the strength of this type of friction material, a number of flat blocks having steel backs attached thereto were made in a die measuring 3¾" x 4½" from a mixture consisting of 72% by weight iron powder, 18% by weight graphite powder and 10% by weight lead powder. They were all cold compacted under a pressure of 14 tons per square inch, heated for 1 hour and hot formed as indicated, cooled with Dry Ice as previously set forth and transverse rupture strength test specimens cut from each were tested with the indicated results.

TABLE I

| Temp.,<br>° F. | Hot<br>Forming<br>Pressure,<br>p.s.i. | Cycle            |                   | No. of<br>Cycles | T.R.S.,<br>p.s.i. |
|----------------|---------------------------------------|------------------|-------------------|------------------|-------------------|
|                |                                       | Time On,<br>sec. | Time Off,<br>sec. |                  |                   |
| 1,900          | 3,000                                 | 7.5              | 1                 | 8                | 18,550            |
| 1,900          | 3,000                                 | 4                | 1                 | 16               | 12,710            |
| 1,800          | 3,000                                 | 4                | 1                 | 16               | 14,200            |
| 1,700          | 3,000                                 | 4                | 1                 | 16               | 7,600             |
| 1,800          | 1,500                                 | 4                | 1                 | 16               | 6,009             |

From the foregoing, it is apparent that there is a relationship between the various variables involved which indicates that the higher temperature of 1900° F., the higher forming pressure of 3,000 pounds per square inch and the 7.5 second on to 1 second off cycle for 8 cycles combine to produce optimum transverse rupture strength. This is also borne out by the comparative rupture strength of the previous examples.

As might be expected, variations in composition of these materials have an effect upon their friction and wear properties and to some extent upon their strength, which is illustrated in the following tables.

TABLE 2

| 10 | Composition, Percent by Weight |          |     |     |                  |         |      |
|----|--------------------------------|----------|-----|-----|------------------|---------|------|
|    | Fe                             | Graphite | Pb  | SiC | MoS <sub>2</sub> | Mullite | Sn   |
| A  | 68.4                           | 17.1     | 9.5 | 5.0 | —                | —       | —    |
| B  | 69.5                           | 16.0     | 5.0 | —   | 2.0              | 5.0     | 2.5  |
| C  | 66.3                           | 15.2     | 9.5 | —   | 1.9              | 4.7     | 2.4  |
| D  | 68.7                           | 2.45     | 4.9 | —   | 1.9              | 19.6    | 2.45 |

TABLE 3

|   | T.R.S., p.s.i. | M.C.F. | Wear, Cu. In. |
|---|----------------|--------|---------------|
| A | 8,050          | 0.49   | 1.83          |
| B | 9,600          | 0.42   | 1.75          |
| C | 9,350          | 0.39   | 1.5           |
| D | 12,600         | 0.22   | 5.0           |

As is evident from inspection, Table 2 illustrates the 30 compositional variables. Segmental brake shoes were made from each of these materials in the same manner as set forth in Example 3 and tested as set forth in Examples 1 and 3. The results of these tests are shown in Table 3.

From the foregoing disclosure it will be apparent that 35 useful railroad brake shoes may be manufactured from compositions which are essentially iron powder and powdered graphite which have much higher strengths and frictional and wear properties which are compatible to or better in some respects than the properties of existing 40 composition shoes and which possess advantages which the composition shoes cannot match.

While for the purposes of this disclosure, certain specific examples have been set forth, it is to be understood that this invention is not to be limited thereby in any way except as set forth in the appended claims. For example, one obvious variation in the processing would be to form the cold pressed compact with the steel backing member in the die or to omit the steel back member completely during the hot forming operation.

Hence, while preferred embodiments have been illustrated and described, it is to be understood that these are capable of variation and modification.

We claim:

1. A method of producing a railroad brake shoe having a body presenting an effective wear portion of compacted and sintered particles consisting essentially of from about 60 to about 75 percent by weight iron powder, from about 10 to about 25 percent by weight graphite powder and up to about 20 percent by weight of powdered friction and augmenting agents, said portion of the shoe having a mean coefficient of friction of at least 0.30 and a wear rate of less than 3.85 cubic inches per 100,000,000 foot pounds of absorbent energy as determined under A.A.R. dynamometer test procedures, comprising: 60 heating the body of compacted and sintered particles to at least 1700° F. and subjecting the heated body to a pressure of about 3000 pounds per square inch applied through a plurality of pressure-no pressure cycles for a time not exceeding 1.5 minutes while the body is confined within a die.

2. A method according to claim 1 wherein the pressure-no pressure cycles involve the application of about 3000 pounds per square inch for a period of up to 10 seconds followed by a period during which no pressure is applied for about 1 second.

3. A method according to claim 2 in which pressure is applied for about 7.5 seconds, in which the total number of cycles is 8, and in which the temperature of the body subjected to pressure is in the range of about 1800° F. to 1900° F.

4. A method according to claim 1 in which the powders consist essentially of from about 65 to 72 percent by weight of iron, about 10 to 20 percent by weight of graphite, up to about 20 percent by weight of lead, up to about 5 percent by weight of tin, up to about 10 percent by weight of Alundum, up to about 7.5 percent by weight of silicon carbide, up to about 20 percent by weight of mullite, and up to about 5 percent by weight of molybdenum disulphide.

5. A method according to claim 3 in which the powders consist of about 70 to 71 percent iron, 2 to 3 percent tin, 1 to 3 percent lead, 4 to 6 percent Alundum, and from 19 to 21 percent graphite.

## References Cited

## UNITED STATES PATENTS

|              |         |                   |            |          |
|--------------|---------|-------------------|------------|----------|
| 2,470,269    | 5/1949  | Schaefer          | -----      | 75-206 X |
| 2,892,707    | 6/1959  | Biggs             | -----      | 75-208   |
| 5 2,899,740  | 8/1959  | Cox               | -----      | 29-182.8 |
| 2,938,790    | 5/1960  | Stedman et al.    | -----      | 75-206   |
| 2,945,291    | 7/1960  | Ankeny et al.     | -----      | 29-182.5 |
| 2,945,292    | 7/1960  | Luther et al.     | -----      | 75-208 X |
| 3,087,814    | 4/1963  | Smiley            | -----      | 75-208 X |
| 10 3,101,527 | 8/1963  | Weinman et al.    | -----      | 75-201 X |
| 3,160,502    | 12/1964 | Quartullo         | -----      | 75-226 X |
| 3,264,726    | 8/1966  | Storchheim et al. | 29-420.5 X |          |
| 3,306,715    | 2/1967  | Schlomer et al.   | -----      | 75-201 X |

15. CARL D. QUARFORTH, *Primary Examiner.*

R. L. GRUDZIECKI, *Assistant Examiner.*